

Oct. 31, 1967

A. ALMAR-NAESS

3,350,288

METHOD FOR CORROSION PROTECTION

Filed April 15, 1964

2 Sheets-Sheet 1

Fig. 1.



Fig. 2



INVENTOR.  
ALMAR ALMAR-NAESS

BY *Kurt Kelman*

AGENT

Oct. 31, 1967

A. ALMAR-NAESS

3,350,288

METHOD FOR CORROSION PROTECTION

Filed April 15, 1964

2 Sheets-Sheet 2

Fig. 3



Fig. 4



INVENTOR.  
ALMAR ALMAR-NAESS

BY  
Kurt Kelman  
AGENT

# United States Patent Office

3,350,288

Patented Oct. 31, 1967

1

3,350,288

**METHOD FOR CORROSION PROTECTION**  
Almar Almar-Naess, Frydenbergveien 12,  
Trondheim, Norway  
Filed Apr. 15, 1964, Ser. No. 360,000  
Claims priority, application Norway, Apr. 27, 1963,  
148,454  
3 Claims. (Cl. 204—147)

## ABSTRACT OF THE DISCLOSURE

Cathodic protection and cleaning of a drying cylinder of a paper-making machine is achieved by applying a negative charge to the cylinder, fixedly arranging an electrode adjacent a portion of the surface of the cylinder which is not covered by the paper web being dried on the cylinder, applying a positive charge to this electrode, pressing an electrolyte through the gap between the electrode and the cylinder surface, and passing a current between the electrode and this cylinder surface.

The present invention relates to a method for corrosion protection and cleaning of a drying roller of a paper-making machine.

It is known that a high degree of protection of a metal or a metal alloy against corrosion may be achieved by making the metal electrically negative in relation to the surrounding electrolyte. This is the principle of cathodic corrosion protection. The potential difference may be obtained e.g. by an outside source of potential, or by a more or less permanent anode, such as for example when a buried pipe is protected. It is usually assumed that the magnitude of the potential difference between the metal and the adjacent liquid layer determines the degree of protection obtained. A uniform protection of the surface, therefore, means a uniform potential difference, which again means a uniform current density on the surface.

A uniform current density on the surface is not always obtainable. The current density is, inter alia, dependent upon the placing of the anode. In the cathodic protection of pipes, as mentioned, the anodes may be distributed in any desired manner and there is no difficulty in obtaining a uniform current density at least as long as the conductivity of the soil is reasonably uniform. If, however, the outside of a ship is to be protected, the anodes are usually distributed along the side of the ship, whereby the current density close to the anode becomes much greater than that further away from it.

In paper making, a wet paper web is brought into contact with the surface of the drying roller at one point and leaves the roller surface at another point remote from the one point, leaving an uncovered roller surface between the one and the other point. The surface of the drying roller is cathodically protected against corrosion and cleaned in accordance with the invention by electrically connecting the drying roller to a negative pole of a direct current source, arranging an electrode in a fixed position with respect to the axis of the drying roller and adjacent a portion of the uncovered roller surface, a gap being defined between the electrode and the uncovered roller surface portion, pressing an electrolyte through this gap, electrically connecting the electrode to a positive pole of the direct current source, and passing a current between the electrode and the uncovered roller surface portion whereby hydrogen gas is evolved on the surface of the drying roller.

The invention is described with reference to the accompanying drawing in which,

2

FIGURE 1 is a schematic vertical section of a drying drum for crystallizing solids,

FIGURE 2 is a schematic vertical section of a Yankee cylinder of a paper-making machine,

FIGURE 3 is a vertical section on a larger scale of the anode arrangement 14 of FIGURE 2, and

FIGURE 4 shows diagrammatically the relationship between the electric current and the overvoltage obtained and employed according to the invention.

10 A rotating drum which is partly in contact with a liquid, as shown schematically in FIGURE 1, can not be protected readily according to the known cathodic principle, as a current can be passed only through that part of the drum which is submerged in the liquid.

15 FIGURE 1 shows a drum 1 for crystallizing solid materials from a solution 2. The drum is warm, the liquid evaporates from the surface 3, and the solids 5 are scraped off by the drum by scrapers or doctor knives 4.

A corresponding problem arises if it is desired to employ cathodic protection for cylinders for drying paper.

20 FIGURE 2 shows how paper web 12 and felt backing 11 at one point is brought into contact with, and at another point remote from the one point leaves, the surface of a Yankee cylinder 10 which may be considered 25 to be a very simple paper-making machine. The paper has a moisture content of about 50% on contacting the cylinder, and the cylinder will be corroded on that area where the paper is wettest. The rate of corrosion depends, inter alia, upon the salt content of the water.

30 In the method according to the invention, an anode 17 is arranged either in the area where the paper and felt come on to the cylinder in a wet condition, e.g. between the pressure rolls 16 (FIG. 2), or preferably on the dry area of the cylinder, e.g. at 14 between two of the 35 doctor knives 13 designed to remove remnants of paper and possible corrosion products from the cylinder.

As known, the electrolytical double layer between a metal surface and the adjacent electrolyte may be considered a condenser C connected in parallel to a non-linear resistance  $R_V$ , as shown in FIG. 4.  $\epsilon_r$  in the diagram denotes a constant voltage simulating the equilibrium potential between the metal concerned and the electrolyte, and  $\eta$  is the overvoltage.  $\eta$  is defined approximately by Tafel's equation:

45 
$$\eta = a + b \log i_q$$
 wherein  $a$  and  $b$  are constants, and  $i_q$  is the current density on the metal surface. On the equivalent diagram in FIG. 4,  $i_q$  corresponds to the amperage through the resistance,  $i_c$  being zero when the condenser is charged. If the total amperage is considered to be

$$i = i_c + i_q$$

then

55 
$$i = C \frac{d\eta}{dt} + 10^{\frac{\eta-a}{b}}$$

60 
$$C \frac{d\eta}{dt} = i - 10^{\frac{\eta-a}{b}}$$

According to this equation the overvoltage will vary principally as shown in FIG. 4 on switching the current on, and off. It will be seen that the overvoltage remains on the surface for some time after the current has been interrupted, which again means that the metal surface is protected against corrosion for some time after the interruption of the current. This "after-effect period" is in the first instance dependent upon the employed current density, and also, as appears from the equation above, upon the constants  $a$  and  $b$ , and the capacity C of the double layers. Measured values of these quantities show

that in a neutral electrolyte such as 0.2-1% NaCl in water, corrosion resistance is obtained for about 60 seconds after the current interruption at a current density of about 0.1 amp./cm.<sup>2</sup>.

When, an anode 17, e.g. of platinum, is arranged on cylinder 10, pressing against the felt 11 between the two pressure rolls 16, so that the applied current passes the wet felt and wet paper, the whole cylinder 10 will be protected against corrosion. The current density must be adjusted to the cylinder speed, the cylinder material and the acting electrolyte. A corresponding corrosion protection is also achieved if the anode 14 is placed on the dry area of the cylinder between the two knives 13, which is also shown in FIG. 2. A useful anode construction is indicated in FIG. 3. The block 21 is made of some electrically insulating material, 22 is the anode. This may consist of platinum, graphite, lead, or other material which is fairly resistant to an anodic load. Between the anode 22 and the cylinder 25 water 23, 24 having sufficient electrical conductivity, is passed, so that current may pass between them and establish an electrolytic double layer on the surface of the cylinder. If the cylinder is warm, the water will no doubt evaporate therefrom, so that it is dry outside the block 21. It has, however, been found that an overvoltage may still be measured on the cylinder surface at the place where the wet paper and felt come on to the cylinder, or at any other place where the cylinder is moist and a potential measurement is possible. The reason for this fact is at the present not entirely clear. As the double layer is connected with an electrolyte, it is difficult to realize how it can continue to exist when the electrolyte has evaporated. It may be guessed that the apparently dry cylinder surface is still covered by a layer of water molecules. It may also be assumed that the double layer is formed between the metal and a thin layer of metal oxide, or that an ion migration takes place in the oxide layer so that the equilibrium potential is changed. The invention is, however, not limited to any specific theory.

If the cylinder is contaminated by an oxide layer, this will, under certain conditions, be dissolved by the cathodic charge. A cylinder of steel or cast iron, for example will normally be coated by a layer of rust wherein the iron is present in the trivalent state, and, therefore, is insoluble in water. By a cathodic charge the trivalent iron is reduced to the divalent state wherein it is soluble in the anode water and it is consequently removed with this. After some time of operation, such a cylinder will, therefore, be cleaned of rust.

The primary electrochemical reaction on the cylinder is hydrogen evolution. The hydrogen loosens burnt-on paper remnants from the cylinder, and they are carried away with the anode water. This action is of great importance for a clean cylinder surface, as the fiber and paper remnants can not always be removed by the ordinary scrapers.

If a suitable metal electrolyte is used instead of water between the cylinder and anode, the cylinder may be coated electrolytically with a metal layer which is more resistant to corrosion than the base material. The coating may be made very thin, it may be applied during operation of the cylinder, and possible wear, peeling, and the like, may be repaired during operation.

By making the cylinder 25 the anode in the circuit shown in FIG. 3, and by employing a suitable electrolyte and current density, it is possible to achieve an electro-

lytic polishing of the cylinder surface. By adjusting the electrolyte and the current density the cylinder may in this way also be protected anodically against corrosion, i.e. the surface is passivated.

It will be appreciated that the foregoing description is only illustrative of the present invention and it is intended that his invention be limited only by the herein-after appended claims.

I claim:

1. An apparatus for corrosion protection and cleaning of the surface of a cylindrical metal drying roller of a paper-making machine, comprising

- (a) the roller,
- (b) a container open on one side,
- 15 (1) the container being arranged water-tightly against the surface of said roller, with the open container side facing the surface,
- (c) an electrode in said container and spaced from the surface,
- (d) means for passing an electrolyte into and out of the container; and

(e) means for passing a direct current between the electrode as the anode and the roller as the cathode.

2. A method for the cathodic corrosion protection and cleaning of a metallic drying roller of a paper-making machine, wherein a wet paper web is brought into contact with the surface of the drying roller at one point and leaves the roller surface at another point remote from the one point, leaving an uncovered roller surface between the one and the other point, the steps of

(1) arranging an electrode in a fixed position with respect to the axis of the drying roller and adjacent a portion of the uncovered roller surface,

- (a) a gap being defined between the electrode and the uncovered roller surface portion,
- (2) passing an electrolyte through said gap,
- (3) passing a direct current between said electrode as the anode and said uncovered roller surface portion as the cathode.

3. The method of claim 2, further comprising the steps of confining said electrolyte in a chamber, one wall of said chamber being the uncovered roller surface portion and another chamber wall being said electrode, and maintaining a water-tight seal between said chamber and said uncovered roller surface portion.

#### References Cited

##### UNITED STATES PATENTS

|           |         |                |       |           |
|-----------|---------|----------------|-------|-----------|
| 1,746,964 | 2/1930  | Polatsik       | ----- | 204-149   |
| 2,847,375 | 8/1958  | Murphy         | ----- | 204-197   |
| 3,025,790 | 3/1962  | Larsen         | ----- | 101-149.2 |
| 3,063,921 | 11/1962 | Leibowitz      | ----- | 204-110   |
| 3,166,487 | 1/1965  | Owren          | ----- | 204-196   |
| 3,193,450 | 7/1965  | Herbert et al. | ----- | 162-192   |
| 3,196,101 | 7/1965  | Hosford        | ----- | 204-196   |
| 3,201,335 | 8/1965  | MacNab et al.  | ----- | 204-147   |
| 3,231,480 | 1/1966  | Collins        | ----- | 204-147   |
| 3,242,064 | 3/1966  | Byrne          | ----- | 204-196   |
| 3,254,012 | 5/1966  | Ziegler        | ----- | 204-147   |

##### FOREIGN PATENTS

|         |        |          |
|---------|--------|----------|
| 449,079 | 9/1927 | Germany. |
|---------|--------|----------|

JOHN H. MACK, Primary Examiner.

T. TUNG, Assistant Examiner.